

Nov. 22, 1955

J. D. WALLACE

2,724,171

ACTIVATION OF FERROELECTRICS

Filed Dec. 11, 1953



Fig. 1



Fig. 2



Fig. 3



INVENTOR.  
JOHN D. WALLACE

BY

  
W. F. Rose  
ATTORNEYS

1

2,724,171

**ACTIVATION OF FERROELECTRICS**

John D. Wallace, Oreland, Pa.

Application December 11, 1953, Serial No. 397,801

4 Claims. (Cl. 29—25.35)

(Granted under Title 35, U. S. Code (1952), sec. 266)

The invention described herein may be manufactured and used by or for the Government of the United States of America for governmental purposes without the payment of any royalties thereon or therefor.

This invention relates to a new method for activating ferroelectrics to impart to them electromechanical properties and to the product produced by the method.

Broadly, the process of the invention comprises subjecting ferroelectric materials to an external, electric field to produce materials of increased dielectric constant and having enhanced electromechanical properties. This procedure is referred to herein as activating the ferroelectric.

Previous methods directed to activating ferroelectrics are based on the premise that the effect produced is due to a crystal realignment which may be effected by application of a voltage stress. For example, one prior art method comprises activating titanate ceramics by the application of high voltages at room temperature, and another method comprises the activation of barium titanate ceramic by the application of a voltage at the transition point of the material, both methods apparently based on the theory that a crystal realignment is effected by the voltage stress produced. These and other conventional methods are indicative of the fact that current criterion has apparently never been considered a factor in activating ferroelectrics.

Former methods for activating ferroelectrics are subject to the disadvantages that they do not produce a uniformly activated product or a completely activated product, due, mainly to the fact that without a consideration of current criteria there is no basis for control of the degree of activation of the material. Incomplete or non-uniform activation results in a relatively small increase in dielectric constant in the material as well as inferior electromechanical properties. Former methods lack reproducibility and also leave certain improvements to be desired in the product, such as higher coupling coefficient and improved hysteresis properties.

It is therefore an object of this invention to provide an improved method for activating ferroelectrics.

It is another object of the invention to provide a method for activating ferroelectric materials which is reproducible and by which complete activation may be obtained.

It is a further object of this invention to provide an activated ferroelectric product for use as an electromechanical element having enhanced electromechanical properties, an increased dielectric constant, a high coupling coefficient and improved hysteresis characteristics.

It has been found that the above and other objects are accomplished in the preferred modification of the invention by the application of an optimum activation current to ferroelectric material at about its transition temperature, and maintaining this current substantially constant as the material cools, preferably to a point at least 65° below the transition temperature.

In the accompanying drawings which are incorporated

2

as a part of this application as an aid in illustrating the application of the invention to titanate ceramic,

Fig. 1 is an isometric view of a cylindrical transducer of barium titanate ceramic;

5 Fig. 2 is a graph illustrating the percent increase in dielectric constant in barium titanate ceramic elements resulting from activation by the present process;

Fig. 3 shows a sampling of hysteresis loops made from data obtained on transducers activated by the method of 10 the invention, and

Fig. 4 shows a sampling of hysteresis loops made from data obtained on transducers activated by a former "voltage" method.

The invention is illustrated in the specification and 15 drawings by its application to barium titanate base ceramic, however, it is equally applicable to any ferroelectric ceramic, and particularly to titanate ceramics. Examples of other suitable materials are, titanates of other metals such as the alkali metals and other alkaline 20 earth metals, niobates, and tantalates of alkali and alkaline earth metals and mixtures of all of the above. Additional specific materials to which the invention is applicable are, tungstenates, bismuth oxides, strontium cerate, boron phosphate, arsenic sesquioxide, lithium ferrite, 25 lithium sulfate and antimony iodide. The ceramics to which the invention applies may comprise 100% of a single ferroelectric or mixtures of ferroelectrics, to which also may be added a minor percentage of various ferroelectric additives for tailoring specific properties. Examples of these additives are calcium titanate, calcium 30 zirconate, strontium titanate, lead titanate, barium titanate and combinations thereof.

For the purpose of this application the transition temperature is the temperature at which the first crystal 35 transformation above room temperature is effected. In the case of barium titanate, for example, it is the temperature at which the crystal structure changes from tetragonal to cubic. As used in the specification and claims 40 the transition temperature of the ceramic is to be interpreted to mean the transition temperature of the ferroelectric crystals contained in the ceramic. To ensure complete transformation, the material being activated is usually heated to about 10° C. above the transition temperature. This temperature is conventionally determined 45 for any material by peaking the dielectric constant of the material.

The optimum activation current has been found to be 50 that amount of current which effects the greatest change in dielectric constant between unactivated and activated material, and is a function of the cross sectional area of the material taken normal to the direction of polarization. It has been discovered that the percentage change in dielectric constant of a ferroelectric material upon activation is proportional to the degree of activation produced in the material. This relationship between the change in dielectric constant and the degree of activation of a material is an important factor in the invention.

Activating current is necessarily expressed in terms of 55 current per square inch of electrode surface for the particular material. The optimum activation current is conveniently obtained by maximizing the change in dielectric constant through activation using sample pieces of the material which have been electrode. That is, the material is subjected to the present process using various amounts of current until that amount of current is found 60 which produces the largest change in dielectric constant.

It is believed that the reason for the effectiveness of the instant method is as follows: It is well established 65 that the desired anisotropy of barium titanate is accomplished by the permanent displacement of the central titanium atom in the crystal lattice in the direction of oxygen atoms. According to the present invention, suffi-

cient energy is provided throughout activation to hold the potential energy of the titanium atom at a constant value corresponding to a position near one of the oxygen atoms in the lattice. This requires furnishing enough energy to move the atom to the new position plus additional energy at a rate which equals its loss in thermal energy. This energy total can be calculated. Accordingly, the present process is based on the supplying of energy in the form of direct current to the element being activated. The amount of current, of course, depends on the size of the material being activated and the degree of activation required. In the preferred embodiment the current is maintained constant during the process by raising the voltage as the resistance increases with decrease in temperature of the material.

As an aid in illustrating the invention reference is made to Fig. 1. The ceramic cylinder 10 was made by slip casting a composition of barium titanate, water and deflocculant and firing the formed casting to vitrification. However, various conventional processes may be used for making the ferroelectric ceramic elements. The electroded surfaces 11 and 12 are of glass base liquid silver and were applied by spraying on the silver and firing to approximately 1500° F. Leads 13 and 14 were then soldered on opposite electroded surfaces as shown using a 2% silver solder.

Activation of cylinders to produce transducers was accomplished as follows: a number of cylinders of barium titanate base ceramic were immersed in chlorinated biphenyl, a high resistance liquid, and slowly heated to a temperature about 10° C. above the transition temperature, this temperature being about 120° C. for barium titanate. Using an RA-38 rectifier power supply furnishing a maximum voltage and current, the current was applied through the leads and increased gradually until it reached 14 microamperes per square inch of electrode surface, the optimum amount of current for complete activation. This figure was obtained as explained above by maximizing the change in dielectric constant using samples of the material. After a short period, the temperature was lowered slowly and the current maintained constant by increasing the voltage as the pieces cooled to a temperature about 65° C. below the transition temperature. The current may be maintained substantially constant until the piece has cooled to room temperature, however, the above temperature is ordinarily an adequate minimum. After cooling, the biphenyl was removed from the pieces by dipping in acetone.

In operation as a transducer, acoustic waves or other mechanical stimuli striking the cylinder 10 result in the generation of a voltage which is taken off on leads such as those shown at 13 and 14. The device shown in Fig. 1 may also serve as a condenser when properly utilized.

The following tabulation of data obtained during activation of a batch of eight barium titanate cylindrical transducers was selected from a larger amount of similar data to illustrate the operation of the invention. The total current required for the group is shown in the table, a total current of 1.3 milliamperes giving 14 microamperes per square inch of total electrode surface. Activation was conducted over a period of about 90 minutes.

Table I

| Temperature (degrees F.) | Voltage | Total Current (milliamperes) |
|--------------------------|---------|------------------------------|
| 285                      | 300     | 1.0                          |
| 275                      | 300     | 1.3                          |
| 273                      | 500     | 1.5                          |
| 232                      | 1,600   | 1.5                          |
| 222                      | 2,100   | 1.4                          |
| 212                      | 2,600   | 1.4                          |
| 200                      | 3,100   | 1.4                          |
| 193                      | 3,100   | 1.4                          |
| 187                      | 3,700   | 1.4                          |
| 170                      | 3,700   | 1.3                          |
| 162                      | 3,800   | 1.3                          |

The elements used in obtaining the above data showed an average change in dielectric constant of about 19% as a result of the treatment. Activated material gave a coupling coefficient of 25 percent.

Groups of barium titanate ceramic elements were activated by the process of this invention using different current values for each group, their average change in dielectric constant noted and the results tabulated in Table II below. The graph of Fig. 2 was made from the results shown in the table. The elements were cylindrical in shape and the outside surfaces were completely electroded with the exception of the end portions. The ceramic pieces had a composition of 96% barium titanate and 4% lead titanate. They had a height of 1½ inches, an average outside diameter of 1½ inches and an average thickness of ½ inch. The dielectric constant was ascertained as follows: A test bridge was used for obtaining the capacity values. The dielectric constant (*k*) was calculated using the following formula. For tubes:

$$k = \frac{1.417 \times 10^{12} C(d_1 - d_2)}{H(d_1 + d_2)}$$

where *C* is the capacity in farads, *d*<sub>1</sub> is the outside diameter in inches, *d*<sub>2</sub> is the inside diameter in inches and *H* is the height in inches. Groups 1, 2, 4 and 5 contained eight elements each and group 3 contained 36 elements.

Table II

| Group | Current (microamperes) | Percent change in dielectric constant (Average) |
|-------|------------------------|-------------------------------------------------|
| 1     | 7.5                    | 12.0                                            |
| 2     | 12.0                   | 13.8                                            |
| 3     | 14.0                   | 19.7                                            |
| 4     | 16.0                   | 14.2                                            |
| 5     | 17.0                   | 13.6                                            |

The final dielectric constant is somewhat dependent upon the purity of the material, however, the percent change in dielectric constant does not vary appreciably with materials meeting reasonable purity standards.

The results in the above table show that the most effective current for titanate ceramics is a current of 14 microamperes per square inch of electrode surface. Use of this current in the process was found to produce complete activation as evidenced by the graph. However, other current values are shown to be effective, and particularly the range from 7.5 to 20 microamperes. The optimum activation current of 14 microamperes per square inch of electrode surface applies to barium titanate ceramics containing PbTiO<sub>3</sub>, CaTiO<sub>3</sub>, and the stannates and zirconates of barium, lead and calcium as additives. The invention, including the range of current values, is applicable to all ceramics having the perovskite type crystal structure. As the results indicate, the invention is not limited in its application to the optimum activation current alone, but in its broadest aspect includes the application of quanta of current, i. e., activating currents to ferroelectrics under the stated conditions to effect activation through an intra-crystal rearrangement, as contradistinguished from prior methods which were based on the application of voltage directed to effecting a change in crystal orientation through stress.

Neither is the invention in its broadest sense restricted to maintaining the initial current constant during cooling, but it includes varying the current as the material cools, the requirement being that a substantial quantum of current, in the order of several microamperes, be supplied throughout the cooling period.

For purposes of comparison, elements of barium titanate ceramic similar to those used to obtain the results shown above were subjected to a standard "voltage" activation process, i. e., they were subjected to various voltages at the transition temperature and the voltage

maintained substantially constant during cooling. The results are shown in Table III below.

Table III

| Voltage | Percent change in dielectric constant |
|---------|---------------------------------------|
| 3,750   | 14.02                                 |
| 5,000   | 13.6                                  |

A comparison of the results of the standard "voltage" method and the "current" method of this invention shows the effectiveness of the present method, particularly when the optimum activation current is used. Further, the results constitute some evidence that activation is an energy phenomenon accompanied by a change in intra-crystal structure rather than a stress phenomenon accompanied by a realignment of crystals.

The method was found to be highly reproducible, a factor resulting from the use of current rather than voltage criterion as a basis for control of the degree of activation of the material.

For a further comparison of the effectiveness of the two methods, reference is made to Fig. 3 showing hysteresis loops produced by pieces activated by the method of this invention and to Fig. 4 showing hysteresis loops produced by pieces activated by the conventional "voltage" method. The hysteresis loops were observed using an oscilloscope with a standard circuit. The observations recorded in Figs. 3 and 4 were made on the same type of elements for which results are shown in Tables I and II. The elements used for the loops of Fig. 3 were subjected to a drive of 4,000 and 5,000 volts respectively and those of Fig. 4 were subjected to a drive of 2,000 and 2,500 volts respectively. The area under the loops shown in Fig. 3 is quite small as compared to that under the loops of Fig. 4 even though the loops of Fig. 3 were produced with twice the drive of those of Fig. 4, indicating a significant difference in power loss to hysteresis in the pieces activated by the two methods.

The product of the invention as illustrated in Fig. 1, when properly utilized, may serve in various applications other than transducers, such as, frequency control devices, electromechanical filters, supersonic sound generators, microphones, telephone receivers, phonograph pick-

ups, piezoelectric relays and similar devices. This is evident from the properties set forth above.

The method of the invention provides a product highly suitable for electromechanical applications as well as for applications based on a change in dielectric constant of the material. The method ensures a high degree of activation as well as favorable hysteresis properties in the product, and is reproducible.

Obviously many modifications and variations of the present invention are possible in the light of the above teachings. It is therefore to be understood that within the scope of the appended claims the invention may be practiced otherwise than as specifically described.

What is claimed is:

1. The method of activating a ferroelectric ceramic which comprises applying electrodes to opposite sides of the ceramic, applying to the ceramic at approximately its transition temperature direct current within a range of about 7 to about 20 microamperes per square inch of electrode surface, and maintaining the supply of current substantially constant until the ceramic cools.
2. The method of activating a ferroelectric ceramic which comprises applying electrodes to opposite sides of the ceramic, applying to the ceramic at its transition temperature about 14 microamperes of direct current per square inch of electrode surface, and maintaining the supply of current substantially constant as the ceramic cools.
3. The method of making an electromechanical element which comprises subjecting a ferroelectric ceramic to an activating current at approximately the transition temperature of the ceramic and maintaining the activating current substantially constant until the ceramic cools.
4. The method of making an electromechanical element which comprises subjecting a ferroelectric ceramic to an activating current at approximately the transition temperature of the ceramic and maintaining the activating current substantially constant until the ferroelectric ceramic cools to about 65 degrees centigrade below its transition temperature.

## References Cited in the file of this patent

## UNITED STATES PATENTS

- |    |           |        |       |               |
|----|-----------|--------|-------|---------------|
| 45 | 2,486,560 | Gray   | ----- | Nov. 1, 1949  |
|    | 2,538,554 | Cherry | ----- | Jan. 16, 1951 |